

Nov. 29, 1927.

1,650,730

E. L. WATROUS

METHOD FOR METAL COATING WIRE AND THE LIKE

Original Filed Sept. 20, 1919

Fig. 1.



Fig. 2.



Fig. 3.



Fig. 4.



Inventor:

Edward L. Watrous,  
(deceased)  
Agnes B. Watrous,  
(Executor)  
by Wallace R. Lane  
*Atty.*

Patented Nov. 29, 1927.

1,650,730

# UNITED STATES PATENT OFFICE.

EDWARD L. WATROUS, DECEASED, LATE OF EL PASO, TEXAS, BY AGNES E. WATROUS,  
EXECUTRIX, OF EVANSTON, ILLINOIS.

## METHOD FOR METAL COATING WIRE AND THE LIKE.

Original application filed September 20, 1919, Serial No. 325,255. Divided and this application filed June 22, 1923. Serial No. 647,006.

The present invention relates to metal coating of objects, such as wire and wire like metal material, barbed wire, wire fabric, chain, woven wire fencing, and the like, and it is to be understood that the term "wire" used in the specification and the claims is generic to all such materials.

This is a division of application Serial No. 325,255, filed September 20, 1919, now 10 Patent No. 1,462,589, for apparatus for metal coating wire, chain, woven wire fencing, and the like.

Among the objects of the invention are to so wind the material to be coated that the 15 parts thereof will be spaced to permit the ready casting-off of excess coating metal and to prevent their adhering when the coating congeals; to space the convolutions of the 20 wire or the like while winding the same for holding the same in spaced and separated condition during the coating operation; to insert or interpose spacers, preferably in the 25 form of rods, between the convolutions as the material is wound so as to provide for the spaces mentioned; to cast off the excess coating metal, preferably by centrifugal action, while the coating metal is still in molten condition and while the material is being 30 held in spaced relation; to wind the material on an open work frame for providing for ready access of the coating metal to the material and the ready passage of the excess 35 metal during the casting-off operation; and such other and further objects, advantages and capabilities as will later more fully appear and are inherently possessed by the invention.

In the drawings illustrating a preferred 40 means for carrying out the invention, Fig. 1 is a perspective view of an open work frame or reel upon which the material may be wound; Fig. 2 is an end view of the same; Fig. 3 is a transverse sectional view showing a part of wound material, and Fig. 4 is a 45 side view of a means for causing centrifugal action together with a part sectional view of means for catching the cast off metal.

The invention contemplates the use of a 50 suitable reel or the like upon which lengthy materials, such as wire, chain, woven wire fencing, and the like may be wound or wrapped, after which the reel with the

wound material may be immersed in a bath of molten metal or spelter or other suitable 55 and desirable material, the reel and contents then being removed from the bath and placed upon a rotatable spindle of a centrifugal machine to operate with sufficient speed to cast off or hurl, by centrifugal 60 force, excess molten metal while the same is still in molten condition for the purpose of leaving a smooth uniform coating upon the wire or the like. The cast off metal may be caught by a shield preferably surrounding the centrifugal machine. After 65 the centrifugal machine is brought to a stop the wire or similar material may be unwound from the reel and bundled for shipment as desired.

Referring now more particularly to the drawings, one form of device for carrying out the invention, is shown as comprising a reel having four corner angle bars 1 spaced from each other to form an open 70 barrel of square cross-section. These angle bars extend the full length of the drum or barrel and have secured thereto at their respective ends, as clearly shown in Fig. 1 of the drawings, pairs of parallel spaced apart angle bars 2 and 3 which have in turn secured to them at right angles thereto pairs of parallel spaced apart angle bars 4 and 5 respectively, they being so connected as to provide outwardly projecting arms at each 75 end of the reel whereby the wound material may be confined between the arms at the respective ends of the drum or barrel of the reel.

Within the open drum may be enclosed a 80 metal sheathing 6 which may be suitably secured within the angles of the angle irons 1 and of utility to prevent the entry of spelter within the interior of the drum and coming into contact with the spindle of the 85 centrifugal machine whereby it may become congealed and adhere to the same.

In order that the turns of wire and the like will not lie flat or close to the surface of the sheathing 6, the reel may be provided 90 with longitudinal angle bars 7 connected to a central portion of the cross bars 2, 3, 4, and 5 intermediate the projecting end portions or arms of angle bars 4, 5, 2, and 3 respectively, as clearly shown in Fig. 1 of 95 the drawings. All of the parts may be con-

nected together by any suitable means such as by riveting or by spot welding or the like.

The object of these bars 7 is to give the drum or barrel a substantially octagonal cross-section thus relieving the wire or like material of kinks.

Where the material to be wound would have the strands closely lying near to each other whereby the spelter would not have as free access to the inner strands or convolutions, and the casting-off of the surplus spelter when subjecting the material to centrifugal action would be more difficult, a spacing means may be provided to hold the convolutions in spaced relation when being wound and treated. For this purpose the reel is provided with a plurality of slotted plates 20 and 21 circumferentially spaced and secured at the inner ends thereof, as by rivets, spot welding or the like, at the intersection of the angle bars 2 and 4 and the angle bars 3 and 5, as clearly shown in Fig. 1 of the drawings. As will be apparent the slotted portions extend substantially at about 45° from the outwardly extending ends of the angle bars to which the plates are attached. The slots 22 and 23 of these plates are preferably open at their outer ends for the ready introduction of rods 24 to act as spacers. These spacing rods extend longitudinally of the reel and are inserted and placed in the slots of two longitudinally aligned plates 20 and 21 as the coils or convolutions of the wire are being wound upon the reel. Preferably, the wire is laid on with one or two layers so that there is substantially no contact between the adjacent portions of the wire and then a set of rods 24 may be inserted and placed so that the successive layers may pass over them. The procedure may continue in the same manner until the reel is filled or the material completely wound thereon. The end of the wire may be secured in any desirable manner to the reel to prevent its unwinding.

With the material properly wound on the reel, the reel together with the material is then immersed in a suitable bath of molten metal or spelter and permitted to remain there until the wire is thoroughly heated and the spelter has had a chance to flow in all around the wire. The reel and coated wire is then rapidly transferred from the spelter bath and placed upon a spindle 25 of a cen-

trifugal machine. The spindle 25 is preferably of the same cross-sectional form as the interior of the sheathing 6 of the reel. The spindle is fast to a shaft 26 suitably driven by gears 27 and 28, driven from a shaft 29 carrying power pulley 30, capable of being driven by a belt or a like means. Around the spindle 25 is preferably provided a shield 31 capable of receiving the cast off metal. During the centrifugal action of the machine the excess or superfluous spelter will be cast off from the wire and caught by the shield 31 and the coating on the wire will remain smooth and uniform.

While I have herein described and shown upon the drawings one form of means for carrying out the invention it is understood that the invention is susceptible of being carried out by other means and also of being modified and changed without departing from the spirit of the invention.

Having now described my invention, I claim:—

1. The method of coating metal wire comprising applying a coating of molten metal to the wire and then subjecting said wire to the action of centrifugal force before the coating metal congeals, said steps being carried out while convolutions of the wire are positively maintained out of contact with other convolutions by means of interposed spacers, so that superfluous coating metal may be freely cast off and adherence of the convolutions prevented when the coating congeals.

2. The method of coating metal wire comprising immersing a reel of wire in a bath of molten coating metal and permitting it to remain therein until the wire is thoroughly heated and the coating metal has flowed in and around the same, and then subjecting the wire to centrifugal action to cast off surplus coating metal before said metal congeals, said steps being carried out while portions of the convolutions of the wire are positively maintained out of contact with contiguous portions of other convolutions, so that adherence of said convolutions will be prevented when the coating thereof congeals.

In witness whereof, I hereunto subscribe my name to this specification.

AGNES B. WATROUS,  
*Executrix of the Will of Edward L. Watrous, Deceased.*